

# UNITED STATES PATENT OFFICE.

ALBERT E. STRIPPEL, OF NEW YORK, N. Y., ASSIGNOR OF ONE-HALF TO MARY E. WALLACE, OF NEW YORK, N. Y.

## STENCIL FABRIC AND PROCESS OF PRODUCING THE SAME.

1,092,509.

Specification of Letters Patent.

Patented Apr. 7, 1914.

No Drawing.

Application filed July 1, 1913. Serial No. 776,893.

*To all whom it may concern:*

Be it known that I, ALBERT E. STRIPPEL, a citizen of the United States, and resident of the borough of Manhattan, in the city and

5 State of New York, have invented a new and useful Improvement in Stencil Fabrics and Processes of Producing the Same, of which the following is a specification.

The objects of my invention are to produce 10 a stencil fabric which will be very durable and sufficiently strong to withstand the severe treatment to which it is subjected in use; which will prevent the type for cutting the stencils from cutting completely 15 through the fabric and blocking out closed characters and which will provide a clear print.

The fabric which is most suitable to be treated to render it desirable as a stencil 20 fabric is a long fiber fabric such as is commonly used in this art, as, for instance, Japanese dental paper.

This fabric may be used either in a single thickness or a multiple thickness as desired 25 and it is pasted along one edge in the usual manner upon a suitable holder of waterproof material for convenience in handling the fabric during its treatment. After the fabric has been completed ready for use it may 30 be cut into the required sizes for use and cemented on the usual cardboard or fiber frames.

The stencil fabric consists of a long fiber fabric provided with a hygroscopic film rendered impervious to the action of the oils contained in printing inks. While this would produce a stencil fabric which could be used for a short time, still to produce a durable stencil it is necessary to keep this film in a 40 soft and pliable state and also to protect it from deterioration for otherwise it would become brittle and crack when handled or run through an addressing machine and it would also be subject to decay. This stencil fabric 45 has heretofore been treated with an organic oil and a preservative as, for instance, glycerin and formaldehyde.

The object of this invention is to produce 50 a stencil fabric which will be superior to those heretofore produced as to pliability, durability and strength. This result is accomplished by the use of metallic salts which are perfectly soluble in water and inorganic acids but not in organic oils so that they 55 will not be affected by the ink solutions.

This method of preservation by the use of metallic salts has proved to be much superior to the former preservation method above referred to.

Where a solution containing gelatin and 60 bichromate of potash is subjected to the presence of light, it has a tendency to thicken, due to the chemical action between the gelatin and the chrome salt whereby the gelatin is rendered insoluble. Heretofore, to 65 keep this solution in a good working degree of fluidity, it has been necessary to exclude it from the action of light which makes the process very difficult and expensive. I have discovered that by the use of a hygroscopic 70 nitrate, such as sodium nitrate, I can expose the solution to the light and yet keep the specific gravity of the solution practically constant for the reason that the nitrate has the effect of materially retarding the setting 75 of the film. The nitrate is not affected by the setting of the film and in the finished product it aids in keeping the paper moist by drawing moisture from the atmosphere along with the chlorid. It also preserves 80 the paper from deterioration by the action of microbes which is the only natural process by which the gelatin and glycerin can be destroyed.

In producing a stencil fabric where the 85 same has to be moistened, before being used, the process is carried out as follows: I dissolve 16 ounces of a colloid of animal origin, such as gelatin, in 5 pints of water and heat the same up to approximately 140° F., and 90 maintain the solution at this temperature as, for instance, in a water bath. Should the gelatin have a tendency to leave an insoluble residue, it is desirable to strain the solution. After the gelatin has been thoroughly dis- 95 solved, I add thereto from 18 to 22 ounces of glycerin and 1.5 ounces of a hygroscopic nitrate, such as sodium nitrate, and mix the parts thoroughly. In a separate vessel I dissolve from .48 of an ounce to .32 of an 100 ounce of a chrome salt, such as bichromate of potash, in 5 pints of water so that the weight of the chrome salt will be between 3½% and 3% of the weight of the gelatin. The smaller the percentage of chrome salt, 105 the softer will be the setting of the film. This solution is heated to 140° F., and added to the solution of gelatin, glycerin and sodium nitrate.

The sheet of long fiber fabric to be treated 110

is run through the solution and given a thorough saturation. The excess is then removed from the fabric by any suitable means, such as rollers and scrapers, one or both. The sheet is then hung up to dry for about twenty-four hours. After the drying and setting of the film has taken place, the sheet is placed upon a suitable non-porous surface, such as glass, and a solution of 5 glycerin is applied thereto by any suitable means, such as a brush or roller. To this solution of glycerin I may add alcohol and aluminum chlorid. The solution which I have found very suitable is one comprising 10 substantially the following proportions, by weight: water, 16 parts; glycerin, 5 parts; alcohol, 1 part; and aluminum chlorid, 1 part. The sheet is then again hung up to dry and may thereafter be cut 15 into the required sizes for use.

What I claim is:—

1. The process of producing a stencil fabric which consists in treating a long fiber fabric with a solution of a colloid of animal 25 origin, glycerin, a hydroscopic nitrate and a chrome salt.

2. The process of producing a stencil fabric which consists in treating a long fiber fabric with a solution of gelatin, glycerin, sodium nitrate and bichromate of potash.

3. The process of producing a stencil fabric which consists in treating a long fiber fabric with a solution of gelatin, glycerin, sodium nitrate and bichromate of potash in 35 substantially the following proportions, by weight; gelatin, 16 ounces; glycerin, 18 to 22 ounces; sodium nitrate, 1.5 ounces and bichromate of potash, .48 to .32 of an ounce.

4. The process of producing a stencil fabric which consists in treating a long fiber fabric, first, with a solution of a colloid of animal origin, glycerin, a hydroscopic nitrate and a chrome salt; second, drying the fabric; third, applying thereto a solution of 45 glycerin; and fourth, again drying the fabric.

5. The process of producing a stencil fabric which consists in treating a long fiber fabric, first, with a solution of a colloid of animal origin, glycerin, a hydroscopic nitrate and a chrome salt; second, drying the fabric; third, applying thereto a solution of glycerin, alcohol and aluminum chlorid; and fourth, again drying the fabric.

6. The process of producing a stencil fabric which consists in treating a long fiber fabric, first, with a solution of a colloid of animal origin, glycerin, a hydroscopic nitrate and a chrome salt; second, drying the 60 fabric; third, applying thereto a solution of glycerin, alcohol and aluminum chlorid in substantially the following proportions, by weight; glycerin, 5 parts; alcohol, 1 part and aluminum chlorid, 1 part; and fourth, again drying the fabric.

7. The process of producing a stencil fabric which consists in treating a long fiber fabric, first, with a solution of gelatin, glycerin, sodium nitrate and bichromate of potash; second, drying the fabric; third, applying thereto a solution of glycerin; and fourth, again drying the fabric.

8. The process of producing a stencil fabric which consists in treating a long fiber fabric, first, with a solution of gelatin, glycerin, sodium nitrate and bichromate of potash; second, drying the fabric; third, applying thereto a solution of glycerin, alcohol and aluminum chlorid; and fourth, again drying the fabric.

9. The process of producing a stencil fabric which consists in treating a long fiber fabric, first, with a solution of gelatin, glycerin, sodium nitrate and bichromate of potash; second, drying the fabric; third, applying thereto a solution of glycerin, alcohol and aluminum chlorid in substantially the following proportions, by weight; glycerin, 5 parts; alcohol, 1 part; aluminum chlorid, 1 part; and fourth, again drying the fabric.

10. The process of producing a stencil fabric which consists in treating a long fiber fabric, first, with a solution of gelatin, glycerin, sodium nitrate and bichromate of potash in substantially the following proportions, by weight; gelatin, 16 ounces; glycerin, 18 to 22 ounces; sodium nitrate, 1.5 ounces and bichromate of potash, .48 to .32 of an ounce; second, drying the fabric; third, applying thereto a solution of glycerin; and fourth, again drying the fabric.

11. The process of producing a stencil fabric which consists in treating a long fiber fabric, first, with a solution of gelatin, glycerin, sodium nitrate and bichromate of potash in substantially the following proportions, by weight; gelatin, 16 ounces; glycerin, 18 to 22 ounces; sodium nitrate, 1.5 ounces and bichromate of potash, .48 to .32 of an ounce; second, drying the fabric; third, applying thereto a solution of glycerin, alcohol and aluminum chlorid; and fourth, again drying the fabric.

12. The process of producing a stencil fabric which consists in treating a long fiber fabric, first, with a solution of gelatin, glycerin, sodium nitrate and bichromate of potash in substantially the following proportions, by weight; gelatin, 16 ounces; glycerin, 18 to 22 ounces; sodium nitrate, 1.5 ounces and bichromate of potash, .48 to .32 of an ounce; second, drying the fabric; third, applying thereto a solution of glycerin, alcohol and aluminum chlorid in substantially the following proportions, by weight; glycerin, 5 parts; alcohol 1 part; aluminum chlorid, 1 part; and fourth, again drying the fabric.

13. A stencil fabric consisting of a long

fiber fabric treated with a solution of colloid of animal origin, glycerin, a hydroscopic nitrate and a chrome salt.

14. A stencil fabric consisting of a long fiber fabric treated with a solution of gelatin, glycerin, sodium nitrate and bichromate of potash.

15. A long fiber fabric treated with solutions of colloid of animal origin, glycerin, a hydroscopic nitrate, a chrome salt, alcohol and aluminum chlorid.

16. A stencil fabric consisting of a long

fiber fabric treated with solutions of gelatin, glycerin, sodium nitrate, bichromate of potash, alcohol and aluminum chlorid.

In testimony that I claim the foregoing as my invention, I have signed my name in presence of two witnesses, this twenty-sixth day of June 1913.

ALBERT E. STRIPPEL.

Witnesses:

F. GEORGE BARRY,  
C. S. SUNDGREN